

Aug. 23, 1932.

R. H. JOHNSON

1,872,745

## PROCESS OF MAKING GUN WAD MATERIAL

Filed March 24, 1930.

Fig. 1



Fig. 20



Fig. 3



Inventor

Reginald H. Johnson

१३४

Drake & French

Attorneys

## UNITED STATES PATENT OFFICE

REGINALD H. JOHNSON, OF MAPLEWOOD, NEW JERSEY, ASSIGNOR TO AMERICAN HAIR & FELT COMPANY, OF CHICAGO, ILLINOIS, A CORPORATION OF DELAWARE

## PROCESS OF MAKING GUN WAD MATERIAL

Application filed March 24, 1930. Serial No. 438,514.

The invention relates to gun wad felt and to a method of producing the same.

It has heretofore been proposed to make gun wads of punched felt, preferably with 5 a reinforced fabric, and in the manufacture of such felt it has been the practice to impregnate the felt produced by a needle-punching loom with sizing, run this felt through driers and thereafter press the same. It has 10 been found with such a procedure that the hair or fibres stick up from the body of the wad material and in order to use the material in the shell-loading machines it has been necessary to coat both sides of the material 15 with paper before cutting the same into wads. This paper coating increases the cost of the product and the waste after cutting has little commercial value because of the necessity for removing the paper. The object of the present 20 invention is to provide an improved gun wad felt and a process of making the same whereby the fibres will be held down in the body of the material so that the same as a finished product may be cut directly into 25 wads and fed to the loading machines.

The invention further consists in the several features hereinafter set forth and more particularly defined by claims at the conclusion hereof.

30 In the drawing Fig. 1 is a diagrammatic view of part of the apparatus used in carrying out the process;

Fig. 2 is a detail, diagrammatic, sectional view through one of the driers.

35 Fig. 3 is a detail view showing certain modifications in the apparatus.

The felt itself is produced by laying a bat or bats of animal hair upon a fabric, such as burlap, and punch-felting the fibres thereto 40 by the use of the usual needle-punching loom and then laying a bat or bats of animal hair upon the opposite side of said fabric and punch-felting the fibres of this bat or these bats to said fabric and to the previously 45 punched fibres by the use of the needle-punching loom, the same preferably being carried out as a continuous process. This provides a material in which a great portion of the fibres extend normal to the plane of the surface 50 of the material, which, in the case of

wads for cartridges, has been found to possess decided advantages as offering a more effective seal for the gases generated on the firing of the cartridge.

According to the present process this 55 punched felt material, designated by the numeral 4, is next run into a tank 5 containing a suitable sizing and during its passage through said tank is impregnated therewith and thence proceeds through a pair of squeeze 60 rolls 6, for removing excess size, to and around a series of steam-heated pressing and drying rolls 7, as shown in Fig. 1, and thence through one or more drying chambers 8 where it is given its final drying subsequent to its 65 finishing treatment.

The drying chambers 8, of course, depend upon the circulation of heated air for the proper drying of the material and a typical 70 form of dryer has been shown in detail in Fig. 2, wherein the material 4 is carried on an endless foraminous belt 9 through the drying chamber and during its progress therethrough is subjected to currents of drying air which, as shown by the arrows, are 75 caused to circulate through the material by means of fans 10 operating in ducts 11 communicating with the upper and lower portions of the drying chamber and at spaced intervals throughout its length. Where, as 80

in previous practice, the size-impregnated wad material is led directly to the drying chamber 8, it has been found that the air passing through the material tends to drive the size from the upper surface and that 85 gravity and air currents acting on the material prevents the sizing from thereafter holding down the protruding fibres. By the present process the passage of the material over the drying rolls 7, which, as shown in the 90 drawing, are arranged to act on opposite sides thereof, acts to smooth down the protruding fibres and also to produce a preliminary surface drying to form a skin coating, preventing the free discharge of the 95 sizing material, as noted above, during its passage through the main driers, such as the chambers 8. Thus, after passing over the rolls 7 the top and bottom sides of the material are in such a condition that as the 100

material is passed through the driers 8 neither the air currents nor gravity will disturb these previously treated surfaces. The result is that after drying the wad material is in a condition in which the usual protruding fibres have been laid down so that they will not cause trouble in the finished product and so that no special coating of paper or other material is necessary in order that the material, as gun wads, may be fed to or used in the loading machines.

In place of the rolls 7, I may, as shown in Fig. 3, use a single large, heated drying and pressing cylinder 12 which acts more particularly on the under side of the material before its passage to the driers and in conjunction therewith or separate therefrom I may use a substantially flat, galvanized iron ironing plate 13, either heated or unheated, as desired, to smooth down the protruding fibres, the material also passing over guide rollers 6'. Either or both of these alternatives will act to prevent the free discharge of the sizing from the material during drying, it being noted that the dragging of the material over the cylinder 12 or the plate 13 puts a smoothing pressure on the same.

After passing through the driers 8 the material is subjected to considerable pressure in hydraulic presses to further pack or compress the felt to the proper thickness and density and as a preliminary to this operation the dried material, in sheet form, is placed in a steam chamber to moisten it somewhat and is then placed between the steam-heated platens of the hydraulic press and the pressure is applied, the movement of these platens being restricted to within the desired thickness dimensions of the material. After this pressing operation the material is ready for use and by the present process the treatment of the sized material is such that, as previously noted, it can be cut into wads and used directly in the loading machines.

It is, of course, to be understood that the invention is not to be limited to any particular form or details of apparatus hereinbefore set forth, or that it is to be otherwise limited to the details above set forth except insofar as such limitations are included in the appended claims.

What I claim as my invention is:

1. In the process of making gun wad material, the step of subjecting a size-impregnated wad material after sizing to the smoothing action of a surface over which the material is passed prior to drying to prevent free discharge of the size through the lower surface of the material during drying.
2. In a process for making gun wad material, the step of subjecting a size-impregnated felt wad material after sizing to heat and pressure to smooth down the protruding fibres and produce a preliminary surface drying to form a skin coating preventing the free dis-

charge of the size from the body of the material during the final stage of the drying process.

3. In a process for making gun wad material, the step of passing a size-impregnated felt wad material after sizing over a series of heated rolls to smooth down the protruding fibres and produce a preliminary surface drying to form a skin coating preventing the free discharge of the size from the material during subsequent drying of the body of the material.

4. The method of making gun wad material which comprises impregnating a previously formed gun wad felt with size, subjecting the size-impregnated material to a pressing and skin-coating drying, thereafter drying the body of the material, and then subjecting the dried material to heat and pressure to further compress it to the desired thickness and density.

In testimony whereof, I affix my signature.

REGINALD H. JOHNSON.

90

95

100

105

110

115

120

125

130